

March 31, 1959

S. KOOPAL

2,880,069

MANUFACTURE OF CALCIUM CARBIDE IN SHAFT FURNACE

2 Sheets-Sheet 1

Filed May 5, 1955

FIG.2



FIG.3



FIG.1

INVENTOR:

*Sids Koopal,  
By Cushman, Darby & Cushman  
ATTORNEYS.*

March 31, 1959

S. KOOPAL

2,880,069

MANUFACTURE OF CALCIUM CARBIDE IN SHAFT FURNACE

Filed May 5, 1955

2 Sheets-Sheet 2

FIG.4



INVENTOR:

*Sidcs Koopal,  
BY Cushman, Darby & Cushman  
ATTORNEYS.*

2,880,069

## MANUFACTURE OF CALCIUM CARBIDE IN SHAFT FURNACE

Sieds Koopal, Sittard, Netherlands, assignor to Stamicarbon N.V., Heerlen, Netherlands

Application May 5, 1955, Serial No. 506,333

Claims priority, application Netherlands May 7, 1954

6 Claims. (Cl. 23—208)

The present invention relates to novel improvements in the manufacture of calcium carbide in a shaft furnace by burning therein, i.e., heat reacting, a solid fuel which consists essentially of carbon, preferably coke, and lime or limestone which is also referred to hereinafter as lime. The high temperature and energy needed for the carbide formation is produced by burning part of the carbon present with an oxygen-rich blast which is injected into the hearth of the furnace through tuyeres, the carbide formed being discharged in the liquid state from the bottom of the furnace, while the gas produced therein is discharged through the furnace top. (See, for example, U.S. patent application Serial No. 302,614, filed August 4, 1952, now abandoned.)

When operating in the manner described above, using thoroughly mixed charges of, for example, one part of lime and two parts of coke, it has been found that carbide with a  $\text{CaC}_2$  content of 60–70% can be continuously prepared if a small furnace (such as one having an internal diameter of 56 cm. and a bed height of 2.5 m.) is used. However, when using a larger furnace (e.g., internal diameter 80 cm., height of bed 2.5 m.) under otherwise identical operation conditions, certain unexpected difficulties are encountered. For instance, it has been found that due to a shell formation consisting substantially of lime over, and partly in front of, the burners, the condition of the hearth is deteriorated to such an extent that hardly any carbide can be produced.

Accordingly, the principal object of the present invention is to provide novel improvements in the abovementioned process whereby said difficulties, and particularly undesired shell formation, are avoided. Other objects will also be hereinafter apparent from the ensuing description and accompanying drawings.

According to the present invention, the manufacture of calcium carbide by heat reacting lime, as such or in the form of limestone, and a fuel consisting essentially of carbon, in a shaft furnace using a gas blast containing a high oxygen content to gasify the fuel and give the temperature and energy necessary for carbide formation is improved by building up the charge of lime and fuel in the furnace in such a way that the concentration of the lime in a plane immediately above the tuyere mouths will increase from the furnace wall towards the center of the furnace. Preferably, the furnace is so charged that the proportion of lime to coke in the charge increases slowly from the furnace wall inwards to a point located at some distance beyond the tuyere mouths after which the lime concentration rises sharply to a maximum at the center of the furnace.

Variation of the lime concentration in the manner discussed effectively eliminates the undesired shell formation mentioned above. Additionally, it has been found that a substantially more efficient reaction is obtained. These improved results can perhaps be explained by the following discussion. Three distinct regions may be noted in a shaft furnace filled with solid fuel and equipped with tuyeres through which an oxygen-rich blast is in-

jected as a result of the combustion and gasification of the solid fuel. These regions are (1) combustion zone in the vicinity of the tuyeres; (2) an adjacent reduction zone where the  $\text{CO}_2$  formed is reduced to CO by the carbon that has been raised to a high temperature, and (3) an adjoining preheating zone where the rising hot gases heat the descending cold solid fuel by passing in countercurrent relation thereto.

By providing the tuyeres with sight holes, the temperature of the glowing fuel surfaces in front of the tuyere ends may be optically measured and the temperature at the end of the reduction zone (where the temperature of the gas phase is taken to be equal to the temperature of the solid fuel) may then be calculated. It has been found that when coke is gasified in a furnace of this type with a blast composed of 47%, by volume, technical oxygen (i.e. 90% by volume of  $\text{O}_2$  and 10% by volume of  $\text{N}_2$ ) and 53%, by volume, of steam, the optically measured temperature of the glowing fuel surface in front of the burners amounts to about  $1600^\circ \text{C}$ , while a calculation shows that the temperature at the end of the reduction zone will be about  $875^\circ \text{C}$ . At higher oxygen contents this temperature difference decreases.

It is, therefore, surprising to find that if the gasification is effected using an oxygen-steam blast with a very high oxygen content, e.g. 65% to 100% oxygen, by volume, or a blast consisting of oxygen enriched air with at least 35% oxygen the temperature at the end of the reduction zone is considerably higher than the measured temperature of the glowing fuel surface immediately in front of the tuyeres. For example, in a test wherein the blast consisted solely of technical oxygen, the temperature measured at the glowing fuel surface in front of the tuyeres amounted to about  $3400^\circ \text{C}$ , while the temperature at the end of the reduction zone was  $4000^\circ \text{C}$ . Accordingly, if a mixed charge of coke and lime is fed to the furnace and a blast with a very high oxygen content is applied thereto, a lime particle located in the immediate vicinity of the tuyeres may have a temperature of many hundreds of degrees below that of a lime particle in the reduction zone, dependent upon the diameter of the furnace. This can be more clearly understood by reference to the accompanying drawings wherein:

Figures 1 and 2 are diagrammatic views of the effect of furnace diameter on the arrangement of the combustion, reduction and preheating zones; and

Figures 3 and 4 are sectional elevations of furnaces provided with means for controlling the distribution of the charge according to the invention.

Referring more particularly to Figure 1, the furnace shown therein has a small diameter, e.g., one up to 0.5 m., and the space between the tuyeres is shown to be entirely occupied by the combustion zone which is overlain by the reduction zone. Figure 2 shows a furnace with a larger internal diameter, e.g., one of the order of 0.5 m. to 2 m. Consequently, in this case, there is a larger distance between the ends of two opposed tuyeres and, as shown, the space between the tuyeres, in contrast to the situation shown in Figure 1, is not entirely occupied by the combustion zone. Thus, in Figure 2, oxygen supplied through the tuyeres is entirely consumed before reaching the center of the furnace and the reduction zone extends downwards into the region between the two opposed tuyeres.

In the situation illustrated by Figure 1, substantially all descending lime particles will first pass through the entire reduction zone, and they are allowed sufficient time to be heated up to a temperature high enough to react with the carbon at a similar temperature to form the desired carbide. However, in the case shown in Figure 2, part of the lime particles, viz., the particles located over the tuyere ends, do not pass through the reduction zone where

the temperature is highest. Furthermore, the stay of these particles in the combustion zone is relatively short due to the fact that this zone is so small. As a result, the lime particles are not heated up to the high temperature (e.g., 2000 to 2200° C.) needed for the carbide formation. Some carbide is formed at the surface of the lime particles, but these particles are cooled down by the relatively cold gas phase issuing from the tuyeres. The carbide thus solidifies and the lime particles cake together. This accounts for the formation of lime-containing shells in front of and above the tuyeres.

Unlike the lime particles descending through the region adjacent to the furnace wall, the lime particles located further towards the center in the case of Figure 2 travel a relatively long path through the high-temperature regions (reduction zone and/or combustion zone) and while doing so, take up so much heat that they become completely or substantially completely converted into carbide. With furnaces of a large internal diameter (above 2 m.) another difficulty may occur which gives rise to operating troubles. Specifically, the energy set free by the fuel combustion will be largely consumed in the formation of carbide from the lime located between the center and the furnace wall. The amount of energy needed for the carbide formation is so large that in the central region of the furnace there will most probably be an actual shortage of energy. As a result, no carbide formation will occur at the center and a mass of unreacted material will accumulate with all of the undesirable results arising therefrom, such as a reduction of the furnace capacity and an obstructed passage of the charge components.

On the other hand, with appropriate modifications, there is the possibility that a carbide with high lime-content, e.g., a carbide containing about 35% by weight of  $\text{CaC}_2$  and having a relatively low melting point (about 1750° C.) can be formed in the central region of the furnace since the formation of such a product requires much less energy. This low-quality carbide at the central region is desirable because in flowing towards the furnace wall, it is in continuous contact with the glowing coke immediately below the combustion zone. In this way, part of the calcium in the impure carbide is converted into carbide and the concentration of carbide is, therefore, increased.

In view of the above considerations, it is of importance, therefore, to adapt the composition of the filling to the locally differing reaction conditions in the furnace when operating with shaft furnaces having an internal diameter of over  $\frac{1}{2}$  m. This is achieved in the manner noted above, i.e., by varying the composition of the carbon-lime mixture from the furnace wall towards the center in such a way that there will first, at the outside, be a region substantially consisting of carbon while in the following regions the lime content will gradually increase toward the center to such a degree that in the central region only so much carbon will be present that a carbide with a high lime content and a low melting point will be formed there. This implies that when the charge used has the usual gross composition of, for example, 20-30% by weight of  $\text{CaO}$  and 80-70% by weight of C (in the form of coke) the lime content may rise, slowly at first and then more rapidly, from 0% by weight of  $\text{CaO}$  at the furnace wall to 85% by weight thereof at the center. As previously noted, this prevents the formation of shells of high lime-content in the vicinity of the tuyere mouths. Additionally, no unreacted charge components will accumulate at the furnace center.

The desired increase in the lime content of the charge towards the center of the furnace may be effected in various ways. For example, use may be made of a special charging installation equipped with a distributing device of such design that the charge can be supplied to the furnace along the wall, through the center or through the intermediate region as desired. A shaft furnace fitted with such a device is illustrated in longitudinal section

in Figure 3 wherein 1 denotes the furnace. The hearth of the furnace is provided with tuyeres 2 connected to a feed pipe for the blast. The walls of the tuyeres and hearth are so designed that they may be protected against unduly high temperatures by means of cooling water.

On the top of the furnace there is mounted a hopper 3 whose contents can be discharged into the furnace by lowering a bell closure 4. Under closure 4 is a distributing device 5, the position of the closure with respect to the distributing device 5 determining the place to which the charge will be delivered. For example, with the bell in position *a*, the charge will descend from the hopper along the outer edge of the bell and the outer wall of the device 5 and will accumulate in an outer 15 region against the furnace wall. On the other hand, when the bell is in position *b*, the charge will pass between the outer edge of the bell and the curved inner wall of the distributing device and accumulate in the central region around the center line. When the bell is put in position *c*, the charge is delivered to the medial 20 region between the central and outer regions aforesaid. By releasing successive quantities of material differing in composition and size into the furnace, a furnace charge can be built up in which the lime content increases, first 25 slowly and then rapidly, from the furnace wall towards the center.

The same result may alternatively be obtained in another way, namely, by making use of the segregation which occurs when the charge is composed of carbon 30 particles and lime particles of different sizes. The specific gravity of carbon in the form of coke is considerably different from that of lime, namely, 0.5 for coke and 1.5 for lime. Accordingly, if a coke-lime mixture, in which the lime particles are smaller than the coke particles, is supplied from a hopper through a centrally arranged vertical feed pipe into a furnace with an internal diameter which is a few times larger than that of the feed pipe, the resulting filling will be so composed that the content of heavier smaller particles (lime) increases from the 35 furnace wall towards the center line of the furnace. The larger the difference between the dimensions of the two components, coke and lime, the more pronounced the segregation will be. The relationship of the diameter of the centrally arranged feed pipe and the furnace diameter 40 also has an influence on the ultimate coke-lime distribution in the furnace charge. For example, to obtain the same degree of segregation when the width of the feed pipe is a comparatively large fraction of the diameter of the furnace, the difference between the dimensions 45 of the coke and lime particles must be larger than when use is made of a narrower feed pipe.

A furnace constructed to make use of the aforesaid segregation effect is illustrated in the longitudinal section shown in Figure 4. The installation consists of the furnace chamber proper, designated by the numeral 1, and a superposed hopper 2 from which the discharge of material is regulated by a bell closure 3. When the said bell is lowered, the contents of the hopper drop through a feed pipe 4 into the furnace chamber. The coarser and light particles roll down outwards along the slope of the previously entered charges whereas the smaller and heavier particles tend to descend vertically. Accordingly, when the bunker is filled with a mixture of relatively large-sized coke particles and smaller-sized lime particles, segregation occurs during filling of the furnace 50 by virtue of the fact that the lime has a specific gravity which is three times as large as that of coke, and the composition of the charge changes in such a way that in the central region far more lime is present than in the outer region adjacent to the furnace wall.

The effect of utilizing a lime concentration which increases towards the center line of the furnace, as herein described, is extremely noticeable as evidenced by the following comparative results using a furnace with an internal diameter of no more than 80 cm., a feed pipe

diameter of 40 cm. and a distance from the lower edge of the feed pipe to the tuyere level of 75 cm. The furnace was charged with a mixture of coke and lime particles of the same diameter, viz., 30-40 mm. Particle segregation was insufficient and hardly any carbide was produced using the following conditions:

Composition of the blast:

35% by volume of steam

65% by volume of technical oxygen (contaminated with 10% by volume of  $N_2$ )

Reaction mixture: 1 part by weight of lime and 2 parts by weight of coke

Amount of blast: 500 m.<sup>3</sup> per hour

Entering velocity of the blast: 80 m./sec.

Height of bed over the tuyere mouths: 15 times larger than the coke diameter

In contrast to the foregoing, the above operations were repeated, except that the furnace was fed with a charge comprising coke having a particle diameter of 40-60 mm. and lime with a particle diameter of 10-20 mm. The resulting filling was such that the lime concentration increased inwardly towards the center of the furnace and a carbide with a  $CaC_2$ -content of 60% by weight was continuously produced without any difficulty.

Various modifications in the invention as described above can be made without in any way deviating from the scope thereof as defined in the following claims wherein I claim:

1. In a process for the production of calcium carbide in a vertical shaft furnace in which a charge of lime and carbonaceous fuel is heat reacted while passing downwardly therethrough with a gas blast of high oxygen content introduced into the lower part of said furnace through tuyeres so as to gasify said fuel and provide the

temperature and energy necessary for carbide formation, the improvement which comprises maintaining, in a zone immediately above said tuyeres, a distribution of lime in said charge which gradually and continuously increases from a minimum concentration of lime adjacent the furnace wall to a maximum concentration of lime in the region of the axial line of said furnace by axially feeding a charge of intermixed lime and carbonaceous fuel particles into said furnace wherein the average maximum dimension of said lime particles is less than one-half the size of said fuel particles whereby disposition of a shell formation of lime on the furnace wall adjacent said tuyeres is substantially avoided.

2. The improved process of claim 1 wherein said carbonaceous fuel is coke.

3. The improved process of claim 1 wherein the concentration of lime gradually increases from substantially zero concentration at the sides of the furnace to about 85% by weight at the center.

4. The improved process of claim 1 wherein the concentration of lime increases slowly from the sides of the furnace for a distance and then increases rapidly to about 85% concentration at the center.

5. The improved process of claim 1 where the oxygen content of said blast is from 65 to 100% by volume by using oxygen-steam blast.

6. The improved process of claim 1 wherein the oxygen content of said blast is at least 35% by using as blast oxygen-enriched air.

30  
35  
25  
20  
15  
10  
5

References Cited in the file of this patent

FOREIGN PATENTS

|         |         |               |
|---------|---------|---------------|
| 525,815 | Belgium | Feb. 15, 1954 |
| 501,376 | Canada  | Apr. 13, 1954 |